

## UNITED STATES PATENT OFFICE.

FREDERICK CARL NIEDERHAUSER AND HAYDEN BENJAMIN KLINE, OF CLEVELAND,  
OHIO, ASSIGNORS TO THE INDUSTRIAL RAYON CORPORATION, OF CLEVELAND,  
OHIO.

## PROCESS FOR TREATING CELLULOSIC MATERIAL.

No Drawing.

Application filed September 20, 1927. Serial No. 220,834.

This invention relates to improvements in the treatment of viscose filaments and products to enhance their dyeing properties, and consists in the introduction of small amounts of inorganic salts in the precipitating or setting bath in the formation of viscose which compounds by their presence cause the finished viscose rayon or product to dye more uniformly and with greater depth or shade of color by the use of dyestuffs and coloring matters normally employed for this purpose. We are familiar with the use of such salts as the compounds of iron, chromium, etc. in the dyeing of cellulosic materials, but they form no claim in this invention. Copper salts have found to be unsuitable in our hands for this purpose on account of producing streaks in bleaching, causing uneven dyeing and for other reasons. Metals, which like lead form highly insoluble sulfates are inapplicable. We have found the best results obtained in our process for increasing the evenness of dyeing of viscose rayon and viscose products by the use of a water-soluble zinc salt, or a zinc salt, compound or derivative which may be transformed into a water-soluble state, and of the zinc salts, their value for this purpose, in general is in proportion to their ready solubility in water or in the solutions or mixtures constituting the various setting baths usually employed in viscose filament manufacture. The use of zinc carbonate is not advised, due to the evolution of carbondioxide from the inorganic acid normally present in the precipitating bath.

It is not material as to the composition in ingredients or their proportion present in the setting bath for the viscose, the addition thereto of relatively small amounts of zinc, zinc compounds or derivatives, we have obtained excellent results in evenness of dyeing when but 0.02% of zinc in solution was present in the precipitating or setting bath in which the viscose was coagulated. However, in general, we prefer to employ larger amounts, preferably up to about 0.9% of elemental zinc by weight to 100 parts by weight of the spin bath. As is well known to those conversant with the art of viscose

manufacture, there is wide variation in physical properties of various batches or runs of viscose at the point where it is coagulated or precipitated, depending upon the degree and length of time of ripening or maturing of the alkali-cellulose and afterwards of the xanthated cellulose, so that a fixed optimum amount of zinc in solution cannot be stated by us at the present moment to obtain the maximum of evenness and exhaustion from bath in the subsequent dyeing of the viscose which has been precipitated in the presence of the relatively minute amount of zinc in solution.

The method of introduction of the zinc salt into the setting bath is relatively unimportant, either a solid salt introduced directly where the solubility, like zinc sulfate, is high, or, the salt may be dissolved separately and added to the viscose setting bath in amounts desired to obtain the dyeing results required.

The percentage of zinc found in the finished viscose rayon when treated by our process varies with the efficiency of the subsequent washing steps and the type of finishing process used. The percentage of zinc remaining in the washed and bleached yarn has no important bearing on the effect produced in the finished fiber toward dyestuffs and coloring matters. That is, the amount of zinc retained in the viscose filament or fiber may be nearly indistinguishable analytically, and still the peculiar and advantageous effect in respect to dyeing remains. It would appear that the minute amounts of zinc, acting catalytically, or otherwise, may change the constitution of the regenerated cellulose sufficient to exhibit the enhanced reactivity to coloring matters, and especially affinity for a large range of dyestuffs. Of the dyestuffs especially applicable to our process are the Indanthrene group, direct dyes and developed colors. It has been noticed that upon introduction into the setting bath of zinc in solution in the relatively small amounts specified, the subsequent bleaching process invariably produces a whiter cellulosic material. The bleaching and desulfurizing steps in the process of

producing viscose rayon, are not materially modified by the introduction of the zinc in solution in the amounts found especially useful by us.

- 5 In connection with the manufacture of viscose filaments which are afterwards to be dyed, there is distinct economies effected in the amount of dyestuff required to produce a given depth of shade, because when zinc is 10 used in the step of the process indicated and in substantially within the limits stated, viscose yarn or film will dye to a deeper shade with the same amount of dyestuff, on account of more nearly complete exhaustion of the 15 dyebath, where the viscose has been coagulated in a normal setting bath to which has been added small amounts of zinc in solution. It should be emphasized that treatment of viscose by our process as herein stated does 20 not result in an inferior product after bleaching, nor is there observable a marked decrease in the tenacity and other desirable characteristics of the finished filament, fiber or film.
- 25 The remarkable dyeing properties exhibited are far out of proportion to the amount of zinc which is retained in the finished product, we having demonstrated that zinc introduced into the finished fiber in the manner herein described, when as little as 10 to 30 20 parts per million of zinc is found in the ash, such yarn will dye many shades darker than will yarn spun in the same manner from a portion of ripened viscose which 35 has been precipitated in a bath not containing zinc, but otherwise of identical composition.

It has been demonstrated by us that the effect of zinc in solution applied as above 40 described is not the effect of a zinc salt utilized as a "mordant", experiments having shown that zinc introduced into the finished fiber from solution does not affect materially the dyeing characteristics of the yarn. This 45 statement in our experience, holds true for as high concentrations as equivalent to 0.7% elemental zinc in the finished fiber.

It would appear that the presence of zinc in the amounts advocated herein, in the bath 50 used for precipitation of the ripened viscose exerts a specific effect resulting in a variation in the character, agglomeration or configuration of the micells or cellulose structural entities. This variation in intrinsic composition is not alone manifested in the specific 55 character of the cellulosic material towards dyestuffs, but is further exemplified in the physical characteristics of the yarn. For instance, the extensibility of viscose rayon is 60 constantly increased by the presence of small amounts of zinc in the spinning solution, and it has been pointed out in many instances in the literature, that increased dye absorptive powers are usually accompanied by high 65 cellulosic extensibility.

We are aware of the United States Patent 1,045,731 granted to Sidney S. Napper for a process which "results in superior products and in economy of working" by the use of a coagulating bath containing zinc sulfate and 70 glucose; and we are aware of the British Patent 216,125 granted to L. A. Bergen for the use of magnesium sulfate in combination with a zinc salt. We make no claim to or for the above. 75

Having now described our invention and in what manner the same may be performed, what we claim and desire to secure by Letters Patent is:

1. A process for increasing the levelness and evenness in dyeing of cellulosic material obtained by the precipitation of viscose in an aqueous bath consisting of an inorganic polybasic acid, an alkali metal salt of the same, and containing zinc dissolved therein, 80 the amount of said zinc not exceeding 0.9% of the weight of the precipitating bath, said viscose after precipitation being treated in a known manner of washing, desulfurizing, 85 bleaching and dyeing, as set forth herein. 90

2. A process for increasing the dye absorptive capacity of cellulosic material obtained by the precipitation of viscose in an aqueous bath, consisting in precipitating the viscose in an aqueous bath consisting of a dibasic 95 inorganic acid, an alkali metal salt of the same, and of relatively small amounts of zinc in the dissolved state, then treating said viscose in a known manner, substantially as described herein. 100

3. A method for effecting economy in the dyeing of that form of cellulosic material obtained from the precipitation of solutions containing viscose, comprising introducing the viscose solution into a precipitating bath 105 consisting of sulfuric acid of strength desired, an alkali metal salt of the same, and zinc in solution in amount not exceeding nine-tenths of one percent of zinc based on the weight of the precipitating solution, afterwards treating the precipitated viscose by ways now known, as set forth herein. 110

4. A process for the introduction into cellulosic material such as hydrated cellulose obtained from the coagulation and other treatment of viscose in solution, of small amounts of zinc, comprising precipitating said viscose solution in an aqueous bath consisting of a polybasic inorganic acid, combinations of the same with an alkali metal, and a soluble form of a zinc salt not exceeding 0.9% of zinc based upon the weight of the coagulating bath, afterwards washing, desulfurizing, bleaching, and dyeing the cellulosic material obtained from the precipitation of the viscose, by ways now known as set forth herein. 115 120

5. A process for increasing evenness, levelness, amount of cellulosic material dyed per unit weight of coloring material and desir- 130

able appearance of the finished material, by washing, desulfurizing, bleaching and dyeing the introduction of viscose in solution into a bath consisting of sulfuric acid, a sodium salt known as set forth herein. of the same and zinc in the form of sulfate, 5 the amount of zinc added to the setting bath not exceeding the equivalent of nine-tenths of one percent of zinc in one hundred parts by weight of the setting bath, afterwards

In testimony whereof we have signed our names to this specification.

FREDERICK CARL NIEDERHAUSER.  
HAYDEN BENJAMIN KLINE.